

No. 813,583.

PATENTED FEB. 27, 1906.

C. B. POTTER.

YARN AND PROCESS OF MAKING THE SAME.  
APPLICATION FILED JUNE 13, 1903.

*Fig. 1.*



*Fig. 2.*



*Fig. 3.*



*Fig. 4.*



Witnesses:

J. D. Garfield  
M. S. Crozier

Inventor  
Clifford B. Potter  
by Chapman & Co.  
Attorneys.

# UNITED STATES PATENT OFFICE.

CLIFFORD B. POTTER, OF SPRINGFIELD, MASSACHUSETTS.

## YARN AND PROCESS OF MAKING THE SAME.

No. 813,583.

Specification of Letters Patent.

Patented Feb. 27, 1906.

Application filed June 13, 1903. Serial No. 181,300.

*To all whom it may concern:*

Be it known that I, CLIFFORD B. POTTER, a citizen of the United States of America, residing at Springfield, in the county of 5 Hampden and State of Massachusetts, have invented new and useful Improvements in Yarns and Processes of Making the Same, of which the following is a specification.

This invention relates to the textile art, 10 and it has special reference to yarns and to the process for making the same.

The object of the invention is to provide an improved yarn composed of fibers whose normal lengths are unequal, as of cotton and 15 wool fibers, and to provide an improved method for making the yarn whereby the mixed fibers may be worked on ordinary cotton working machinery regardless of the proportionate quantity of wool fiber in the mixture.

It is well known that in order to work a mixture of cotton and wool fibers on a machine adapted to cotton if the proportion of wool exceeds a certain amount it is impossible 25 to produce a good yarn. This is largely owing to the fact that the wool fibers are very much longer than the cotton fibers. It is also known that in mixing fibers of cotton and wool it is exceedingly difficult to produce a 30 yarn through which the wool is evenly distributed, and it is also difficult to produce a yarn from such mixture of uniform thickness. These difficulties have in a measure been overcome by using some short-fibered wool, 35 such as noils, with the cotton; but the supply of this material is totally inadequate to the demands of the market.

In the drawings forming part of this application, Figure 1 represents a bunch of cotton 40 fibers, and Fig. 2 represents a bunch of woolen fibers; Fig. 3, a portion of a sliver of wool, and Fig. 4 shows two subdivisions of the sliver.

In carrying this invention into practice the 45 length of the cotton fibers which are to constitute a part of the mixture is first ascertained, and it may be assumed that these are represented in Fig. 1 of the drawings. The wool which is to constitute the other portion of 50 the mixture is then run through a suitable machine and drawn into a sliver, as shown in Fig. 3, and this is in turn put through a machine which will cut it up into lengths substantially 55 equal to the length of the cotton fibers which constitute the other portion of the mixture

these lengths being indicated by the portions *a* between the dotted lines *b b*. The normal length of the wool fibers as compared with cotton may be assumed to be shown in Fig. 2. By thus treating the wool the average length 60 of its fibers cannot exceed the average length of the cotton fibers, and the two may be worked together by means of machinery adapted to operate on the normally shorter fiber. It has been found in practice that by 65 thus unifying the length of the fibers a uniform distribution of the wool through the cotton, or vice versa, in the process of manufacture can be relied upon. Furthermore, the uniform length of the fibers results in the production of a yarn possessing great uniformity, 70 whereas when any mixture of two fibers whose lengths are as unequal as those of cotton and wool is made the yarn will be drawn out thin in spots and will remain bunched in other 75 spots.

A still further advantage is possessed by a yarn made under the process herein disclosed, and that advantage consists in the fact that the proportion of wool to cotton may be materially reduced without resulting deterioration in the apparent quality of the fabric made from the yarn. The reason for this is that the soft or woolly feeling which the addition of the wool gives to the fabric or the 80 yarn is due to the projection of the ends of the fibers beyond the surface of the fabric or yarn, and it therefore stands to reason that with an admixture of wool fibers which have been cut into lengths substantially equal to 85 the cotton there will be provided in a given length of yarn a larger number of ends of the wool fibers which may project beyond the surface to produce this soft "feel" in the goods. Another advantage and a very great one resulting from this method consists in the fact that it is immaterial what the proportionate 90 quantities of wool and cotton may be in the mixture if the average lengths of the two fibers be equal, for the mass will work equally well 95 whether the quantity of wool be thirty per cent. of the whole or seventy-five per cent. of the whole, whereas when wool fiber is used which is long as compared with the cotton and the quantity of wool is as much as fifty 100 per cent. great difficulty is experienced in working such a mixture, and it is practically impossible to work it on machinery adapted to cotton and produce a level yarn. It is 105 thus apparent that the range of yarns which 110

may be manufactured by a mill fitted with machinery adapted only to cotton is greatly increased by means of this process.

In carrying out the present invention it is to be understood that it is obviously necessary that the wool fibers be arranged in parallel order prior to the cutting thereof and that the use of the word "sliver" is to be considered in its broadest sense as indicating any grouping of the fibers in such parallel order as to permit their being cut in the manner described. As to the use of the word "wool" herein, this term is to be considered as including all the animal fibers of like nature to wool—that is, inclusive of all the fleece fibers.

Having thus described my invention, what I claim, and desire to secure by Letters Patent of the United States, is—

1. The method of making a cotton and wool yarn which consists in drawing the wool

into a sliver, then mechanically subdividing the latter transversely into sections whose length shall equal substantially the length of the cotton fiber, then mixing the fibers and forming the yarn in the usual manner.

25

2. A yarn composed of cotton and wool fibers, the latter being cut from a sliver into lengths corresponding substantially to the length of the cotton fiber.

3. A yarn composed of cotton and wool fibers, the latter being cut from a sliver into lengths corresponding substantially to the length of the cotton fibers and uniformly distributed therewith throughout the yarn, said wool fibers presenting an extended area of 35 exposed ends.

CLIFFORD B. POTTER.

Witnesses:

K. I. CLEMONS,  
Wm. H. CHAPIN